

# UNITED STATES PATENT OFFICE.

ROBERT ABBOTT HADFIELD, OF SHEFFIELD, ENGLAND.

## MANUFACTURE OF STEEL.

No. 851,233.

Specification of Letters Patent.

Patented April 23, 1907.

Application filed June 18, 1904. Serial No. 213,131.

*To all whom it may concern:*

Be it known that I, ROBERT ABBOTT HADFIELD, a subject of the King of Great Britain, and a resident of Sheffield, county of York, 5 England, have invented certain new and useful Improvements in the Manufacture of Steel, of which the following is a specification.

My invention relates to the manufacture of steel, and has for its purpose to produce a 10 metal particularly adapted for structural and other purposes on account of its high tenacity, very high elastic limit, and great ductility and toughness. To this end I make the steel of a certain composition, as hereinafter 15 fully set forth, using carbon, manganese, nickel, and chromium in proportions within certain limits, as stated below in detail.

A typical example of my steel contains .44% of carbon, .32% of manganese, 3.5% of 20 nickel, and 1.71% of chromium. The proportions may be varied within certain limits, thus I may employ from 10% to 25% more or less carbon than indicated above, and the amount of chromium might vary from about 25 1% to 3%, and the nickel from about 2% to 5%. The percentage of manganese may also be varied but should be kept low so as not to exceed say .25 or .3%.

The steel may be produced in various manners, as by the open-hearth process or in a crucible.

Steel of the composition above set forth has a high tenacity and a very high elastic limit, yet remarkable ductility and toughness. These valuable properties may be enhanced by the following treatment:—

One method of treatment is as follows:— The steel is carefully heated to a temperature between about 750° to 850° centigrade, 40 preferably 785°, and quenched in oil. Then the steel is reheated to a temperature between about 620° and 630° and quenched in water. When so treated the steel has an elastic limit of over 100,000 lbs per square 45 inch and a tensile strength of over 110,000 lbs per square inch.

Another method of treatment is as follows:—The steel is carefully heated to a temperature of 710° centigrade and quenched in 50 oil. Then the steel is reheated to 620° centigrade and quenched in water.

I claim as my invention:

1. The herein described process of producing steel of great strength, which consists in 55 first making steel containing manganese, nickel, and chromium, (the percentage of

manganese being low) heating the steel to a temperature between about 750° to 850° centigrade, quenching in oil, reheating to a temperature between about 620° and 630°, and 60 quenching in water.

2. The herein described process of producing steel of great strength, which consists in first making steel containing manganese, nickel, and chromium, (the percentage of manganese being low) heating the steel to a relatively high temperature below its melting point, quenching in oil, reheating to a temperature below that first employed, and 65 quenching in water. 70

3. The herein described process of producing steel of great strength, which consists in first making steel containing manganese, nickel, and chromium, (the percentage of manganese being low) heating the steel to a 75 relatively high temperature below its melting point, cooling it quickly, reheating to a temperature below that first employed, and again cooling quickly.

4. The herein described process of increasing the strength of steel, containing manganese, nickel and chromium, the percentage of manganese being low which consists in heating it to a temperature between about 750° to 850° centigrade, quenching in oil, reheating to a temperature between about 620° and 630°, and 80 quenching the entire body of the steel in water. 85

5. The herein described process of increasing the strength of steel, containing manganese, nickel and chromium, the percentage of manganese being low which consists in heating it to a relatively high temperature below its melting point, quenching in oil, reheating to a temperature below that first employed, and 90 quenching the entire body of the steel in water. 95

6. The herein described process of increasing the strength of steel, containing manganese, nickel and chromium, the percentage of manganese being low which consists in 100 heating it to a relatively high temperature below its melting point, cooling it quickly, reheating to a temperature below that first employed, and again cooling the entire body of the steel quickly. 105

In testimony whereof I have hereunto set my hand in the presence of two subscribing witnesses.

ROBERT ABBOTT HADFIELD.

Witnesses:

EDWIN MORTIMER,  
H. MARTIN.